

## UNITED STATES PATENT OFFICE.

ALLAN C. SHAVER, OF MONTREAL, QUEBEC, CANADA.

## COMPOSITION FOR REMOVING RUST FROM FABRICS.

No Drawing.

Application filed April 29, 1921. Serial No. 466,495.

*To all whom it may concern:*

Be it known that I, ALLAN C. SHAVER, a subject of the King of Great Britain, and resident of the city of Montreal, in the Province of Quebec and Dominion of Canada, have invented certain new and useful Improvements in Compositions for Removing Rust from Fabrics, of which the following is a full, clear, and exact description.

10 This invention relates to improvements in method of and composition for removing rust from fabrics, and the object of the invention is to provide for the removal of rust very quickly and easily and without any damage to the fabrics.

According to the present invention, the stained portion of fabrics is saturated with a composition containing oxalic acid and oil Gaultheria, and is then subjected to a jet of steam, with the result that the stain is removed immediately and without any damage to the fabric. As soon as the stain is completely eradicated, the fabric is thoroughly rinsed in clean water. The oil exerts a softening influence on the stained portion of the fabric as well as a protective influence on the fabric itself, so that the oxalic acid may remove the stain without danger to the fabric. The action of the acid is imperfect 30 without the application of steam.

The composition used comprises preferably by weight:

|                |     |
|----------------|-----|
| Water          | 94% |
| Oxalic acid    | 5%  |
| Oil Gaultheria | 1%  |

The amount of oil used in proportion to the acid may be considerably increased or decreased but approximately the percentage above indicated will be most satisfactory, as it provides sufficient oil to soften and protect

the fabric without providing an excess of oil. The amount of acid used in proportion to water may also be considerably increased or decreased. Acid may be used sufficient to 45 make a substantially saturated solution which is about 11%, but with the stronger acid solutions a greater amount of oil should be used to protect the fabric. The disadvantage of the stronger solutions is that they 50 are somewhat dangerous in the hands of an unskilled person and that more careful and thorough rinsing is required to remove the acid from the fabric.

Having thus described by invention, what 55 I claim is:

1. A composition for removing rust stains from fabric containing oxalic acid and oil Gaultheria.
  2. A composition for removing rust stains from fabric, comprising an aqueous solution of oxalic acid containing a small amount of oil Gaultheria.
  3. A composition of matter for removing rust stains from fabrics, containing oxalic acid and approximately one-fifth of the weight of the acid of oil Gaultheria.
  4. A composition of matter for removing rust stains comprising an aqueous solution of oxalic acid containing approximately 1% 70 by weight of oil Gaultheria.
  5. A composition of matter for removing rust stains from fabric, containing an unsaturated aqueous solution of oxalic acid containing oil Gaultheria.
  6. A composition of matter for removing rust stains from fabric, comprising by weight approximately 94% of water, 5% of oxalic acid and 1% of oil Gaultheria.
- 75 In witness whereof, I have hereunto set my hand.

ALLAN C. SHAVER.